

# UNITED STATES PATENT OFFICE.

WILLIAM G. ROACH, OF CINCINNATI, OHIO, AND ALBERT C. ROACH,  
OF NEWPORT, KENTUCKY, ASSIGNORS TO THE CINCINNATI CHROME  
LEATHER COMPANY, OF CINCINNATI, OHIO, A CORPORATION OF  
OHIO.

## PROCESS OF TANNING HIDES.

No. 839,205.

Specification of Letters Patent.

Patented Dec. 25, 1906.

Application filed June 15, 1904. Serial No. 212,698.

*To all whom it may concern:*

Be it known that we, WILLIAM G. ROACH, residing at Cincinnati, in the county of Hamilton and State of Ohio, and ALBERT C. ROACH, residing at Newport, in the county of Campbell and State of Kentucky, citizens of the United States, have invented certain new and useful Improvements in Processes of Tanning Hides, of which the following is a specification.

The object of our invention is to provide an improved process for the metallic tanning of hides; and our invention consists in the process hereinafter described and claimed.

The hides are prepared for tanning in the usual way and then placed in a chromic-acid bath until thoroughly permeated by the chromic acid. This bath may consist of four pounds of bichromate of potash, four pounds of hydrochloric acid, and from four to six hundred pounds of water, which will form a chromic-acid bath, as will be readily understood by those skilled in the art.

After the hide has been thoroughly permeated with chromic acid we subject it to a bath of an organic reducing agent, such as glycerin, or glucose, or some other saccharine substance. The proportions of this bath may be five pounds of glucose or other reducing agent to five pounds of water. We allow the hide to become thoroughly saturated with this solution, which will take about thirty minutes.

Under the conditions of application there will be no substantial reducing action between the chromic acid and glucose for a considerable length of time, so that the glucose will uniformly penetrate the hide before any substantial reduction takes place. This per-

mits intimate and uniform association between the chromic acid and glucose before reduction, so that when reduction does take place the chrome-oxid is uniformly deposited on the fibers of the hide. Thus it will be seen that the two substances, glucose and chromic acid, are introduced into the fiber of the hide in a substantially inactive chemical state and become intimately and uniformly associated together and with the fiber of the hide before reduction takes place.

The next step in our process is to remove the hide from the glucose solution and subject it to a bath of hot vapors, such as steam

not under pressure. This may be done by hanging the hides in a room containing steam. A convenient method for introducing the steam to the chamber is by means of steam-supply pipes arranged in any convenient manner in the chamber and provided with holes in their walls adapted to permit escape of the steam into the chamber. The hides are left hanging in the steam-chamber until the chromic acid has been thoroughly reduced. With thin hides this would take about one-half hour and with thicker hides a proportionately longer time. The effect is to cause the chromic acid to be reduced to chrome-oxid, and the conditions are most favorable for causing that oxid to combine thoroughly with the gelatinous substances of the hide. The water-vapors present serve to maintain the softness of the hides during reduction. The reduction taking place uniformly throughout the hides will cause a uniform deposit of chrome-oxid on the fibers, and consequently a uniformly - tanned leather. We are not prepared to state the exact chemical reaction which takes place in the hide; but we have found that the chromic acid is thoroughly reduced and that the chromic oxid combines fully with the gelatinous substances of the hide.

After the hide has undergone this 'afore-said step it is a marketable leather which does not need any further "stuffing" to make it retain its plumbness. This leather is suitable for such purposes as belting, upholstering, and enameled leather.

In cases where it is desired to have a greased leather it may be stuffed in the ordinary manner.

We claim as our invention—

1. The process of tanning hides which consists in introducing into the fibers of the hide, in a substantially inactive chemical state, substances containing the elements of a tanning matter adapted to be released by reaction between said substances, and then subjecting the hides to the action of steam until the reaction takes place, substantially as specified.

2. The process of tanning hides which consists in introducing into the fibers of the hide, in a substantially inactive chemical state, a reducible metallic compound and a reducing agent; and subjecting the hides to the action

of steam until reduction takes place, substantially as specified.

3. The process of tanning hides which consists in introducing into the fibers of the hide, in a substantially inactive chemical state, a reducible metallic compound and an organic reducing agent; and subjecting the hides to the action of steam until reduction takes place, substantially as specified.

10 4. The process of tanning hides which consists in the introduction of chromic acid, then glucose, and then subjecting them to the action of steam, substantially as specified.

15 5. The process of tanning hides which consists in subjecting them to the action of

chromic acid, then of a saccharine solution and then subjecting them to the action of heat in the presence of vapors to promote the reduction of the chromic acid.

6. The process of tanning hides which consists in subjecting them to the action of chromic acid, then to that of a reducing agent and then to the action of steam substantially as described. <sup>20</sup>

WILLIAM G. ROACH.  
ALBERT C. ROACH.

Witnesses:

W. F. MURRAY,  
A. McCORMACK.